

## ALUMINUM BRIGHTENER COMPOSITIONS

Daniel R. Kelly, Wyandotte, Mich., assignor to Wyandotte Chemicals Corporation, Wyandotte, Mich., a corporation of Michigan

No Drawing. Filed Oct. 13, 1958, Ser. No. 766,721

18 Claims. (Cl. 41—42)

This invention relates to ways and means for brightening aluminum surfaces of articles such as the wings of aircraft. More particularly, it relates to aluminum brightener compositions based on methylcellulose as a thickener.

In the manufacture and use of articles having aluminum surfaces (including aluminum alloy surfaces), such as those found, for example, on aircraft, such surfaces become discolored, tarnished and covered with corrosion and oxidation products. For at least aesthetic reasons, it is desirable in many cases to remove such tarnish and corrosion products and discoloration, and otherwise brighten the surface of the aluminum article. A less obvious reason for removing such products of corrosion and oxidation resides in the fact that frequently cleaned aluminum surfaces tend to last longer than infrequently cleaned aluminum surfaces, or, to state it another way, in the fact that corrosion tends to beget corrosion. Consequently, the removal of corrosion products from aluminum articles upon completion of manufacturing operations has become a standard finishing step and the frequent removal of corrosion products from aluminum articles in use has become a standard maintenance procedure, particularly in the aircraft industry.

In many instances, the removal of corrosion products and the like from aluminum and aluminum alloy surfaces can be accomplished merely by immersing the article into a bath of an aqueous solution of a mineral acid and wetting agents, and, when the desired degree of brightening has occurred, by removing the article from the bath, rinsing and then drying. In the case of aircraft, however, it is unwieldy and impractical to dip or immerse the same into baths. Accordingly, it is customary in the aircraft industry to brush or spray the brightener solution on the aluminum surfaces to be brightened and, when the desired degree of brightening has occurred, to rinse the solution from the brightened surface. To prevent run-off and subsequent streaking of vertically disposed surfaces, the brightener solution under these conditions usually comprises a thickening agent, such as methylcellulose, in sufficient concentration to make the solution sufficiently viscous (about 80 to about 200 centipoises at 25° C.) and uniformly adherent to the surface to be brightened.

However, such solutions (particularly those containing methylcellulose as the thickening agent) as have been developed by the art suffer from a major deficiency. They cannot be mass-produced in large quantities and shipped long distances to various points of use nor can they be stored for much more than 1 month for the reason that, as heretofore formulated, the solutions rapidly lose viscosity. This loss in viscosity can be compensated for by initially formulating the solution with a sufficiently higher concentration of thickening agent so that, even though degradation takes place, the solution will have the desired viscosity at a predetermined time of use. However, the raw material cost of such a solution is sufficiently great as to discourage formulators at

long distances from the point of use from supplying these solutions at reasonable prices to users. Moreover, because the storage life of such solutions is limited, users are not able to purchase such solutions in large quantities.

Consequently, up to the time of this invention, it has been customary to prepare the solution only in such quantities as will be used immediately and to do so at or near the place of use.

The aluminum brightener solutions developed heretofore by the art also suffer from another deficiency in that they are corrosive to magnesium and magnesium alloys. There is a tendency more and more for aircraft to be constructed of both aluminum and magnesium parts. Consequently, this problem of corrosion of magnesium surfaces is becoming quite serious. Indeed, the U.S. Air Force in Technical Order, No. 1-1-1C—"Cleaning of Aeronautical Equipment" has stated that "All known brightener agents contain chemicals which attack magnesium and therefore the use of brighteners on aircraft using magnesium necessarily must be curtailed."

Still another deficiency of the prior art aluminum brighteners resides in the fact that they are all in aqueous solution form. Elimination of water from the composition until the time of use would result in savings in shipping and handling costs. Elimination of the water does not, however, solve the problem of excessive loss in viscosity nor does it eliminate the liquid form of the brightener since the strong acids which make up the prior art compositions are liquid at the usual temperature of shipping and storage. Furthermore, I have found that substitution of the strong, liquid acids by water-soluble, solid acids of equal strength or by solid, hydrolyzable acid salts that will produce acids of equal strength in aqueous solution does not prevent excessive degradation of the methylcellulose in the solid formulation and resultant low viscosity of the aqueous solution prepared at the time and place of use.

It is therefore a general object of this invention to provide the art with a dry aluminum brightener composition comprising methylcellulose, which, regardless of its age, will give, upon addition of water, an aluminum brightener solution with a viscosity within the desired range (about 80 to about 200 centipoises at 25° C.).

It is another object of this invention to develop an aluminum brightener composition which is substantially noncorrosive to magnesium and magnesium alloy surfaces.

Still another specific object of this invention is to develop an aluminum brightener composition in solid form, which, regardless of its age, can be readily dissolved in water in a given proportion and give an aqueous solution having a viscosity within the desired range, which is substantially noncorrosive to magnesium and magnesium alloy surfaces.

These and other objects as may appear as this specification proceeds are achieved by this invention.

In summary, my invention comprises a dry aluminum brightener composition consisting essentially of a finely divided mixture of about 10 to about 25 weight percent of a solid, hydrolyzable, acid fluoride salt selected from the group consisting of alkali metal bifluorides, ammonium bifluoride and sodium silicofluoride; about 20 to about 50 weight percent of a solid, water-soluble, organic acid with an ionization constant in the range of about  $1 \times 10^{-4}$  to about  $2 \times 10^{-3}$ ; about 15 to about 30 weight percent of a water-soluble methylcellulose of a viscosity type of about 400 to about 4000 centipoises; and about 10 to about 30 weight percent of a water-soluble, acid-stable wetting agent.

The function of the acid fluoride salt is to provide hydrofluoric acid under conditions of use. Representative acid fluoride salts are ammonium acid fluoride, so-

dium acid fluoride, potassium acid fluoride and the like. Alkali metal, as used herein, refers to the monovalent elements of the first group of the periodic system, such as lithium, sodium, potassium, rubidium and cesium. Although alkali metal silicofluorides give good results when employed in the compositions of the invention, the aforementioned acid fluorides are more effective on heavily oxidized aluminum surfaces.

The concentration limits of the hydrolyzable acid salt are determined primarily by practical considerations. Too low a concentration results under use conditions in a brightening rate too slow for commercial acceptance. Too high a concentration and under use conditions the resultant rate of attack on aluminum becomes intolerable and, if the organic acid concentration is low enough, a white stain will be deposited on the metallic surface.

The organic acid with a dissociation or ionization constant in the range from about  $1 \times 10^{-4}$  up to about  $2 \times 10^{-3}$  functions under use conditions both as a sequestering agent and as an acidifying agent for the release of hydrogen fluoride by the acid fluoride salt. In the case of those organic acids having more than one ionizable hydrogen atom, such as, for example, citric acid, and thus having more than one ionization constant, only the first ionization constant is the significant constant for the purposes of this invention. The ionization constant of the organic acid has been found to be quite critical. If the ionization constant is higher than about  $2 \times 10^{-3}$  the methyl-cellulose degrades too rapidly, not only in solution but even in dry formulation, thereby leading to poor viscosity stability of the brighter composition. An ionization constant less than  $1 \times 10^{-4}$  results in a lower than practical brightening rate.

Organic acids that fall within the defined class and which have been found to be suitable are citric acid, tartaric acid, glycollic acid, and diglycollic acid.

The range of concentration of the organic acid in the dry composition is dependent on the brightening action. The concentration less than the minimum limit results in a brightening rate too low to be acceptable, a brightening action that is rapidly exhausted and white staining of the aluminum surface at higher concentrations of the acid fluoride salt. A concentration greater than the maximum limit will not produce any adverse effect; however, it is a practical limit based on the economics of the composition.

The methylcellulose under use conditions functions as a thickener or viscosity agent. It is well known in the art. Moreover, processes for producing methylcellulose are well known in the art. Methylcellulose is produced and sold according to viscosity type (which is a function of the methoxy content) and degree of purity. In general, technical grade to chemically pure methylcellulose can be used in the practice of this invention. The methylcellulose can be used as such or in the more common, hydroxypropyl modified, form. However, regardless of the degree of purity and the chemical form of the methylcellulose used in the practice of this invention it will usually be of a viscosity type such that a 2% by weight aqueous solution thereof at 20° C. will give an absolute viscosity in the range of about 400 to about 4000 centipoises. A viscosity type below about 400 centipoises results in the minimum proportion of methylcellulose in the compositions of this invention being too large to be practical. The upper limit on the viscosity type is dictated only by the fact larger viscosity types are not at present available in commercial quantities.

The range of concentration of methylcellulose in the composition is determined solely by the desired range of viscosities under use conditions, which range is from about 80 to about 200 centipoises at 25° C. Since there is no substantial degradation of the methylcellulose in the presence of the other components of the compositions

of this invention, no excess methylcellulose is involved in this range of concentration.

The water-soluble, acid-stable wetting agent component of the brightener composition aids in the penetration of the tarnish, etc. by the liberated hydrofluoric acid, as well as a more uniform cleaning action. It also functions to give a fine, stable foam when the composition under use conditions is rinsed from the brightened surfaces. Exemplary of nonionic wetting agents which can be used are (1) alkylarylpolyethers, such as the oxyethylated adducts of nonyl phenol having an oxyethylene content in the range of about 65 to about 85 weight percent of the total molecule and the oxyethylated adducts of tertiary octyl phenol having an oxyethylene content in the range of about 65 to about 75 percent by weight of the molecule, and (2) the polyoxyethylene-polyoxypropylene-polyoxyethylene (EPE) block polymer type of nonionics (see U.S. Patent No. 2,674,619—Lundsted), which are marketed by Wyandotte Chemicals Corporation under the trademark Pluronic, wherein the molecular weight of the polyoxyethylene base is in a range from 800 to about 2500 and the oxyethylene content is from about 30 to about 80 weight percent of the total molecule, which wetting agents are well known in the art. Examples of acid-stable anionic wetting agents which can be employed in the compositions of the invention include (1) the well-known alkylarylsulfonates such as sodium alkylbenzenesulfonate wherein the alkyl group has from about 10 to 18 carbon atoms and (2) the alkylsulfates such as sodium laurylsulfate.

To minimize dust formation during handling of the solid compositions of this invention, a small amount of liquid should be present in the composition. This can be accomplished by using up to 10 weight percent of a liquid nonionic wetting agent in the composition. Beyond 10 weight percent other handling problems, such as caking, are encountered, wherefore, in the solid compositions of this invention, which have a nonionic wetting agent concentration in excess of 10 weight percent, the excess should preferably be a solid nonionic wetting agent. An example of a liquid nonionic wetting agent is one marketed as Triton X-100, which is the oxyethylated adduct of tertiary octyl phenol having an oxyethylene content such that a 1 weight percent aqueous solution has a cloud point of 149° F. Suitable solid nonionic wetting agents are the EPE polyols in which the polyoxypropylene base has a molecular weight in the range of about 800 to about 2500 and an oxyethylene content from about 70 to about 80 weight percent of the total molecule. An example of such an EPE polyol is that marketed under the trademark Pluronic as "F68," in which the molecular weight of the polyoxypropylene base is in a range from about 1500 to about 1800 and the polyoxyethylene content is about 80 weight percent of the total molecule.

To prepare an aluminum brightener solution with the desired viscosity and brightening rate, the dry composition is mixed with sufficient water to produce a solution in which the proportion of composition is from about 2.8 to about 9.5 weight percent and the proportion of water is from about 97.2 to about 90.5 weight percent and the mixing is continued until all of the solid composition has gone into solution.

To facilitate rapid dispersion and hydration of the methylcellulose component of the composition, the water used in making up the solution should be warm to hot. On the other hand, warm to hot water may not always be readily available or practical. Consequently, the solid composition may contain up to about 40 weight percent of a dispersing agent, such as, for example, a water-soluble salt, sugar, urea and the like, which has a preferential affinity for water in the presence of the methylcellulose and which does not produce residues which are corrosive to aluminum. To avoid such residues

the dispersing agent should be substantially free of chlorides, bromides, iodides and strong acids. An example of a suitable water-soluble salt is ammonium sulfate. Although up to 40 weight percent of a dispersing agent gives good results, a preferred concentration is in the range of about 20 to 40 weight percent.

An example of a composition suitable for use in aqueous solution in accordance with the concepts of this invention is as follows:

#### COMPOSITION A

| Components                                                  | Weight Percent |
|-------------------------------------------------------------|----------------|
| Ammonium acid fluoride                                      | 10.0           |
| Citric acid                                                 | 20.0           |
| Methylcellulose (Viscosity type—4,000 cps.)                 | 20.0           |
| Alkylarylpolyether alcohol (Triton X-100) or (Igepal CO630) | 10.0           |
| Ammonium sulfate                                            | 40.0           |

The alkylarylpolyether alcohol identified in the foregoing composition as Triton X-100 has already been described. The polyether identified as Igepal CO630 is an oxyethylated adduct of nonyl phenol which has an oxyethylene content of about 65 weight percent of the total molecule.

To prepare an aluminum brightener solution from Composition A, mix 5 parts by weight of Composition A with 95 parts by weight of water. This composition will be completely in solution in a few minutes, and be ready for use. Moreover, the resultant solution will have viscosity stability over a long period of time.

It has been observed that Composition A in aqueous solution at 25° C. at 5 weight percent concentration results in a solution viscosity of approximately 200 centipoises, at 7 weight percent a solution viscosity of about 600 centipoises and at 12 weight percent a solution viscosity of about 5 centipoises. Below the 12 weight percent concentration the acid concentration of the solution is at a safe level, whereas, above 12 weight percent, the acid concentration of the solution is such as to result in excessive etching of aluminum surfaces. Keeping in mind that the desired range of viscosities for aluminum brighteners under use conditions is about 80 to about 200 centipoises, it will be seen that Composition A has an inherent safety feature in that at unsafe concentrations the resultant solution is too thin to be used. This feature or property is possessed by all of the compositions of this invention.

It has also been observed that when the dry compositions of this invention are placed into aqueous solutions and stored for long periods of time, the solutions display a remarkable degree of viscosity stability.

Accordingly, this invention also involves the concept of liquid concentrates which are prepared by dissolving a solid composition, such as Composition A, in just enough water to completely solubilize the composition. At the time or place of use the concentrate is then diluted with water until the viscosity is in the desired range of about 80 to about 200 centipoises at which dilution the proportion of solids in solution will be less than about 10 weight percent.

In addition, this invention involves the concept of liquid, aluminum brightener compositions that are ready for instant use even after long periods of storage.

Such compositions (liquid concentrate and use solution) consist essentially of about 97 to about 87 parts by weight of water and in solution about 0.8 to 8.5 parts by weight of acidic components consisting of a hydrolyzable acid fluoride salt selected from the group consisting of alkali metal bifluoride salts and ammonium bifluoride, and an organic acid with an ionization constant in the range of about  $1 \times 10^{-4}$  up to about  $2 \times 10^{-3}$  with the mol ratio of said organic acid to said hydrolyzable acid fluoride salt being in a range from about 0.5/1

to 3/1; about 0.8 to about 2 weight percent of a methylcellulose of a viscosity type of about 400 to about 4000 centipoises; and about 0.5 to about 3 weight percent of a nonionic wetting agent. Within these limits of concentration said compositions have an initial viscosity in the range of about 80 to about 3000 centipoises at 25° C., and a viscosity after 6 months from about 80 to about 1500 centipoises at 25° C., and are substantially noncorrosive to magnesium.

10 The concentration ranges for the various components of the liquid brightener composition are established by the same considerations as involved in the case of the dry brightener compositions. However, in the case of the liquid brightener the range of concentrations selected for the organic acid is somewhat narrower than in the case of the dry brightener. The reason for this is that above the maximum limit organic acids with an ionization constant in the higher end of the ionization constant range tend to degrade the methylcellulose in the 15 liquid brightener over long periods of storage. On the other hand the maximum limit can be exceeded in the case of organic acids with ionization constants in the lower end of the range without accelerating the degradation of the methylcellulose. Consequently, the concentration range set forth is an optimum range generally applicable to the liquid brightener compositions of this 20 invention.

To prepare a use solution from a concentrate solution of this invention, dilute with water until the desired viscosity is reached.

An example of a liquid aluminum brightener concentrate of this invention is as follows:

#### COMPOSITION B

| Components                                    | Weight Percent |
|-----------------------------------------------|----------------|
| Ammonium acid fluoride                        | 1.00           |
| Citric acid                                   | 2.00           |
| Methylcellulose (Viscosity Type—4,000 cps.)   | 1.85           |
| Alkylarylpolyether alcohol (Igepal CO630)     | 0.93           |
| EPE nonionic surfactant (Pluronic polyol L64) | 0.92           |
| Water                                         | 93.30          |

45 The alkylarylpolyether alcohol in Composition B has already been described with reference to Composition A. The EPE nonionic surfactant in Composition B is a polyoxyethylene-polyoxypropylene-polyoxyethylene polyol in which the molecular weight of the polyoxypropylene base is in the range of about 1500 to about 1800 and the ethylene oxide content of the molecule is about 40 weight percent.

50 A sample of Composition B has shown an initial viscosity of about 1750 centipoises at 25° C. To use Composition B add 1 part by weight of water to 1 part by weight of Composition B. Such a use solution gave an initial viscosity of 130 centipoises at 25° C.

Unless otherwise indicated, all viscosity measurements reported in this specification were determined at 25° C. 55 with a Brookfield Synchro-Lectric Viscometer, Model 60 LVF (SN2497) using Spindle No. 2 and speeds of 30 r.p.m. up to a viscosity of 1000 cps. and 12 r.p.m. for viscosities over 1000 cps.

To use the aluminum brightener solutions of this 65 invention, the solutions in the desired range of viscosity are merely brushed or sprayed on the surface to be brightened. The viscous solution remains in place and will eventually dry in place unless removed. About 30 seconds after applying the brightener solution, brightening action as evidenced by gas formation can be observed. 70 After about 5 to 20 minutes, depending upon the condition of the oxidized aluminum surface, the brightening composition can be removed therefrom by rinsing the surface with water under pressure from hoses, spray-  
ers and the like.

7  
Example I

This example illustrates the storage stability of the solid compositions of this invention.

A solid, finely divided, composition corresponding to Composition A (using Triton X-100 nonionic) was prepared and stored for approximately a month and a half at 100° F. at normal humidity. A 5 weight percent aqueous solution of a sample of the composition at the time of preparation gave a viscosity measurement of 180 centipoises at room temperature. A 5 weight percent aqueous solution of a sample of the composition taken at the end of the storage period gave a viscosity measurement of 130 centipoises at room temperature.

## Example II

To illustrate the viscosity stability of the solution compositions of this invention various aluminum brightener composition concentrates were prepared and viscosity measurements made. The following tabulated data was obtained.

TABLE I

| Components                                                              | Weight Percent |       |       |       |       |
|-------------------------------------------------------------------------|----------------|-------|-------|-------|-------|
|                                                                         | No. 1          | No. 2 | No. 3 | No. 4 | No. 5 |
| Methylcellulose (Viscosity Type—4,000 cps.)                             | 2.0            | 2.0   | 2.0   | 2.0   | 2.0   |
| Alkylarylpolyether alcohol (Triton X-100)                               | 1.0            | 1.0   | 1.0   | 1.0   | 1.0   |
| EPE nonionic surfactant (Pluronic nonionic L64)                         | 1.0            | 1.0   | 1.0   | 1.0   | 1.0   |
| Hydrofluoric acid                                                       | —              | —     | 2.0   | 2.0   | —     |
| Phosphoric acid                                                         | —              | 6.5   | 1.0   | —     | —     |
| Ammonium acid fluoride                                                  | —              | —     | —     | 1.0   | —     |
| Citric acid                                                             | —              | —     | —     | —     | 2.0   |
| Hydrofluosilicic acid                                                   | —              | —     | —     | —     | —     |
| Water                                                                   | 90.0           | 88.5  | 93.0  | 94.0  | 93.0  |
| Viscosity of fresh solution (centipoises at 25° C.)                     | 2,000          | 2,000 | 2,000 | 2,000 | 2,000 |
| Viscosity of solution after 9 days at 100° F. (centipoises at 25° C.)   | 700            | 105   | 230   | 345   | 975   |
| Viscosity of solution after 30 days at 100° F. (centipoises at 25° C.)  | 275            | 10    | 35    | 60    | 620   |
| pH of an aqueous solution with 5% by weight of formulation after 9 days | 6.4            | 2.5   | 2.8   | 3     | 4.5   |

In the table it will be observed that the best viscosity stability is demonstrated by formulation No. 5, which is the only one within the concepts of this invention, and that the reduction of viscosity in formulation No. 5 is reasonably close to that of the control formulation No. 1 comprising methylcellulose and no acid constituents. Just why the viscosity of the control formulation No. 1 became reduced is not known although it is speculated that bacterial action was involved. However, the data does demonstrate that the presence of the strong acids in formulations Nos. 2, 3 and 4 accelerated the reduction in viscosity.

## Example III

This example illustrates the utility of the compositions of this invention.

The solution composition corresponding to formulation No. 5 in Example II was diluted on a 1 to 1 weight basis with water and then applied to 3 tarnished panels of aluminum alloy (2024-T3 Alclad) which were disposed in a vertical position. In each case, after about 30 seconds, the action of the brightener could be seen by the gassing that occurred at the surface of the aluminum alloy. Five minutes after placing the brightener composition on the panels, the composition was washed off from each of the panels under a stream of water and the condition of each of the exposed surfaces was observed. In each case, the exposed surface of the panel was bright, no streak marks were observed, and no evidences of white deposits or corrosive pitting were to be found.

8  
Example IV

This invention illustrates the substantially non-corrosive action of the compositions of this invention on magnesium surfaces.

Weighed panels of magnesium were immersed for one-half hour in a solution corresponding to formulation No. 5 in Example II, removed, rinsed, dried and then weighed. Weight changes were from plus 0.002 gram to minus 0.001 gram.

A weighed panel of magnesium was immersed in one commercially available, liquid aluminum brightener (Brand A) and another weighed panel of magnesium was immersed in another commercially available aluminum brightener (Brand B). After one-half hour of immersion in each case, the panels were removed, rinsed, dried and weighed. The weight changes were minus 0.080 gram and minus 0.040 gram, respectively.

Thus it can be seen that in accordance with the concepts of this invention aluminum brightener compositions are obtained which not only have the property of good viscosity stability over long periods of time, but which are substantially non-corrosive to magnesium and magnesium alloys.

## Example V

This example illustrates the effect of the ionization constant of the organic acid on the storage stability of the brightener compositions of this invention. It also illustrates that sodium bifluoride may be used in place of ammonium bifluoride in the composition.

TABLE II

| Components                                                                                                                         | Weight Percent |       |       |
|------------------------------------------------------------------------------------------------------------------------------------|----------------|-------|-------|
|                                                                                                                                    | No. 6          | No. 7 | No. 8 |
| Methylcellulose (Viscosity Type—4,000 cps.)                                                                                        | 20             | 20    | 20    |
| Ammonium Sulfate                                                                                                                   | 40             | 40    | 35    |
| Alkylarylpolyether alcohol (Triton X-100)                                                                                          | 10             | 10    | 10    |
| Ammonium Bifluoride                                                                                                                | 10             | —     | 10    |
| Sodium Bifluoride                                                                                                                  | 20             | 20    | —     |
| Citric Acid                                                                                                                        | —              | —     | 20    |
| Sulfamic Acid                                                                                                                      | —              | —     | —     |
| Viscosity of 5% by weight aqueous solution of sample of formulation when first made up (cps.)                                      | 190            | 190   | 170   |
| Viscosity of 5% by weight aqueous solution of sample of formulation after holding for 30 days at 100° F. at normal humidity (cps.) | 155            | 150   | 30    |

Citric acid has a first hydrogen ionization constant of  $8.7 \times 10^{-4}$  whereas sulfamic acid has an ionization constant of  $1.01 \times 10^{-1}$ . It will be observed that the sulfamic acid formulation (No. 8) is not at all stable in storage as compared to the citric acid formulations.

## Example VI

This example illustrates the storage stability of other organic acids having ionization constants within the range of about  $1 \times 10^{-4}$  to about  $2 \times 10^{-3}$ .

TABLE III

| Components                                                                                                                                | Weight Percent |        |        |
|-------------------------------------------------------------------------------------------------------------------------------------------|----------------|--------|--------|
|                                                                                                                                           | No. 9          | No. 10 | No. 11 |
| Methylcellulose (Viscosity Type—4,000 cps.)                                                                                               | 20             | 20     | 20     |
| Ammonium Sulfate                                                                                                                          | 40             | 40     | 40     |
| Ammonium Bifluoride                                                                                                                       | 10             | 10     | 10     |
| Alkylarylpolyether alcohol (Igepal CO-630)                                                                                                | 10             | 10     | 10     |
| Glycolic Acid                                                                                                                             | 20             | —      | —      |
| Citric Acid                                                                                                                               | —              | 20     | —      |
| Diglycolic Acid                                                                                                                           | —              | —      | 20     |
| Viscosity of 5% by weight aqueous solution of sample of formulation after storage for approximately 5 weeks at 100° F. at normal humidity | 120            | 100    | 80     |

Glycolic acid has an ionization constant of  $1.52 \times 10^{-4}$ ,

citric acid has an ionization constant for the first hydrogen of  $8.7 \times 10^{-4}$ , while diglycollic acid has an ionization constant for the first hydrogen of  $1.1 \times 10^{-3}$ . Thus, within the critical range of ionization constants, the solid, finely divided compositions of this invention have storage stability.

It should be understood that as this invention may be embodied in several forms without departing from the spirit or essential characteristics thereof, the embodiments described in this specification are therefore illustrative and not restrictive, since the scope of the invention is defined by the appended claims rather than by the description preceding them, and all changes that fall within the metes and bounds of the claims, or that form their functional as well as conjointly cooperative equivalents, are therefore intended to be embraced by those claims.

Also, the term "consisting essentially of" as used in the definition of ingredients present in the composition or compositions claimed is intended to exclude the presence of significant amounts of other materials in such proportions as to interfere substantially with the properties and characteristics possessed by the compositions set forth while permitting the presence of other materials in such proportions as not substantially to affect adversely said properties and characteristics.

What is claimed is:

1. A finely divided composition suitable for use in aqueous solution at a concentration of about 2.8 to about 9.5 weight percent to brighten aluminum surfaces which consists essentially of (1) about 10 to about 25 weight percent of hydrolyzable acid fluoride salt selected from the group consisting of alkali metal bifluorides, ammonium bifluoride, sodium silicofluoride and mixtures thereof; (2) about 20 to 50 weight percent of water-soluble organic acid with an ionization constant in the range of about  $1 \times 10^{-4}$  up to about  $2 \times 10^{-3}$ ; (3) about 15 to about 30 weight percent of water-soluble methylcellulose of a viscosity type of about 400 to about 4000 centipoises; and (4) about 10 to about 30 weight percent of a water-soluble, acid-stable wetting agent.

2. A composition according to claim 1 wherein said organic acid is citric acid.

3. A composition according to claim 1 wherein said organic acid is tartaric acid.

4. A composition according to claim 1 wherein said organic acid is glycollic acid.

5. A composition according to claim 1 wherein said organic acid is diglycollic acid.

6. A composition according to claim 1 wherein up to about 40 weight percent of said composition constitutes a dispersing agent substantially free of chlorides, bromides, iodides and strong acids.

7. A composition according to claim 6 wherein said dispersing agent comprises sugar.

8. A composition according to claim 6 wherein said dispersing agent comprises urea.

9. A composition according to claim 6 wherein said dispersing agent comprises ammonium sulfate.

10. A composition suitable for use in aqueous solution at a concentration of about 5 parts by weight per 95 parts by weight of water, which consists essentially of about 10% by weight of ammonium acid fluoride, about 20% by weight of citric acid, about 20% by weight of methylcellulose of viscosity type of about 4000 centipoises, about 10% by weight of a water-soluble, acid-stable wetting agent, and about 40% by weight of ammonium sulfate.

- 5 11. An aluminum brightener composition consisting essentially of about 97 to about 87 parts by weight of water and in solution (1) about 0.8 to about 8.5 parts by weight of acidic components consisting of a hydrolyzable acid fluoride salt selected from the group consisting of alkali metal bifluorides and ammonium bifluorides, and an organic acid with an ionization constant in the range from about  $1 \times 10^{-4}$  to about  $2 \times 10^{-3}$  and at a mol ratio to said fluoride salt in a range from 10 about 0.5 to about 3; (2) about 0.8 to about 2 parts by weight of methylcellulose of a viscosity type of about 400 to about 4000 centipoises; and (3) about 0.5 to about 3 parts by weight of a water-soluble, acid-stable wetting agent, which composition is characterized by a 15 viscosity in the range of about 80 to about 3000 centipoises at 25° C.
12. A composition according to claim 11 wherein said organic acid is citric acid.
13. A composition according to claim 11 wherein said 20 organic acid is tartaric acid.
14. A composition according to claim 11 wherein said organic acid is glycollic acid.
15. A composition according to claim 11 wherein said organic acid is diglycollic acid.
- 25 16. An aluminum brightener concentrate suitable for use upon dilution at a 1 to 1 weight ratio with water, which consists essentially of about 93 weight percent of water and in solution (1) about one weight percent of ammonium acid fluoride; (2) about two weight percent 30 of citric acid; (3) about two weight percent of methylcellulose of a viscosity type of about 4000 centipoises; (4) about one weight percent of an alkylarylpolyether alcohol wetting agent; and (5) about one weight percent of a polyoxyethylene-polyoxypropylene-polyoxyethylene 35 nonionic wherein the polyoxypropylene portion of the molecule has a molecular weight in the range of about 800 to about 2500 and wherein the polyoxyethylene oxide content of the total molecule is 70 to 80 weight percent.
- 40 17. A method for brightening a tarnished aluminum surface in conjunction with a magnesium surface wherein the magnesium surface is not substantially damaged, which comprises (1) applying to said surface a viscous liquid consisting essentially of about 97.2 to about 90.5 weight percent of water and in solution about 2.8 to about 9.5 weight percent of a composition consisting 45 essentially of about 10 to about 25 weight percent of a hydrolyzable, acid fluoride salt selected from the group consisting of alkali metal bifluoride, ammonium bifluoride, sodium silicofluoride and mixtures thereof, about 20 to about 50 weight percent of an organic acid with an ionization constant in the range of about  $1 \times 10^{-4}$  to about 50  $2 \times 10^{-3}$ , about 15 to about 30 weight percent of a methylcellulose of a viscosity type of about 400 to about 55 4000 centipoises, and about 10 to about 30 weight percent of a water-soluble, acid-stable wetting agent, said liquid having a viscosity in the range of about 80 to about 200 centipoises at 25° C.; and (2) rinsing said solution from said surface when the tarnish on said surface has been 60 removed therefrom.
- 55 18. A method according to claim 17 wherein the mol ratio of said organic acid to said fluoride salt is in a range of about 0.5/1 to 3/1.

65 References Cited in the file of this patent

UNITED STATES PATENTS

2,687,346 McDonald \_\_\_\_\_ Aug. 24, 1954